

## UNITED STATES PATENT OFFICE.

GEORGE W. SARGENT, OF PITTSBURGH, AND JOSEPH W. WEITZENKORN, OF WASHINGTON, PENNSYLVANIA.

## PROCESS OF RECOVERING MOLYBDENUM FROM MOLYBDENITE.

1,401,924.

Specification of Letters Patent. Patented Dec. 27, 1921.

No Drawing.

Application filed June 14, 1920. Serial No. 388,785.

To all whom it may concern:

Be it known that I, GEORGE W. SARGENT, a resident of Pittsburgh, in the county of Allegheny and State of Pennsylvania, and 5 JOSEPH W. WEITZENKORN, a resident of Washington, in the county of Washington and State of Pennsylvania, have invented a new and useful Improvement in Processes of Recovering Molybdenum from Molybdenite, of which the following is a specification.

The invention relates to the recovery of molybdenum from molybdenite.

Until recently molybdenum has been classed as a rare or semi-rare metal, and its 15 use has been limited to products in which, for the most part, the cost of manufacture is not the controlling or prime factor. Chiefly because the metal was rare and its use so limited, the processes heretofore developed for its recovery from molybdenite, that is to say, molybdenum sulfid ore, are 20 not such as may be used to economically recover the metal in large quantities.

Of late years large deposits of molybdenite have been discovered, so that there are 25 now available sources of molybdenum of such extent that the metal may, if economically recovered from the ore, be extensively used in large quantities for various purposes, as for example in the manufacture of 30 ferrous alloys such as steel and iron.

It is, accordingly, the object of the invention to provide a method whereby molybdenum, substantially free from sulfur, may 35 be economically recovered from molybdenite, and also to provide a method for economically producing directly from molybdenite a molybdenum alloy low in sulfur.

The invention, as far as concerns its 40 broader aspects, is predicated upon our discovery that molybdenite readily combines with an oxid of manganese in an exothermic reaction which evolves almost sufficient heat to render the continued reaction self sustaining after the molybdenite and the metallic oxid have been heated to the reaction temperature.

In the preferred practice of the invention molybdenite is caused to combine with manganese dioxide in the presence of a reducing agent such as carbon, the reaction being carried on at an elevated temperature in any well known or desired type of furnace or crucible. However, the process may be, and

preferably is, practised in an electric furnace of the resistor arc or semi-arc resistor type.

Prior to its being charged into the furnace, the molybdenite, crushed or otherwise reduced to substantially a powder state, is 60 mixed with powdered manganese dioxide and a suitable reducing agent such as carbon in the form of charcoal, coke and the like. When the proper proportions of these materials are used it has been found that at a 65 temperature of about 2000° F. the following reaction takes place:—



It is believed that in the first step in this 70 reaction the manganese dioxide combines exothermically with the molybdenite to form a manganese-molybdenum-sulfid compound, which is thereafter reduced by the carbon. Whatever the steps in the reaction may be, 75 it has been found that carbon dioxide passes off as a gas, that substantially pure molybdenum settles to the bottom of the furnace, and that a low melting point fluid slag of manganese sulfid separates from, and floats 80 upon, the molybdenum.

After the materials have been heated to the temperature required for starting the reaction, the exothermic character of the reaction makes it necessary to apply little if 85 any additional heat. Before tapping the furnace for final cleaning, the molten mass may, if found necessary, be cleaned up by the addition of carbon or manganese or an oxid thereof. However, it has been found that, if the mixture is properly proportioned 90 at the beginning, little if any cleaning up is required, the condition of the slag under proper mix conditions being such that the slag readily throws out the metallic molybdenum, retaining little if any of the metal. 95

If it is desired to recover the molybdenum in the form of a ferro-alloy for subsequent use in the manufacture of alloy steel and iron, iron in the form of filings, turnings, etc., may be placed in the mix, the amount of iron thus added depending upon the proportion of iron and molybdenum desired in the ferro-molybdenum. The process may be otherwise practised as previously described, it having been found that the molten iron readily mixes or alloys with the molten molybdenum so that there results a ferro-

55

60

65

70

75

80

85

90

95

100

105

molybdenum alloy of predetermined proportions obtained directly from the molybdenite.

As thus far described, the process has been explained solely with reference to the use of manganese dioxide and carbon as the materials to be combined with molybdenite in the initial mix. The invention also contemplates, as a step in the process, the combining of an oxid of manganese and molybdenite without carbon. By forming a mix of these two materials and heating it in the manner described, there is eliminated a large portion of the sulfur in the form of sulfur dioxide, and a manganese-molybdenum-sulfid compound is formed, which can be further reduced to metallic molybdenum by the addition of carbon, or which may be used as a starting point to make other molybdenum compounds.

The invention also contemplates the simultaneous recovery of molybdenum from molybdenite and the manufacture of an alloy such as molybdenum steel. For this purpose an oxid of manganese and molybdenite may be charged directly into a steel manufacturing furnace, such as an electric or open hearth furnace. Sufficient carbon to reduce the manganese-molybdenum-sulfid may be introduced with the manganese and molybdenite, or the carbon of the steel-furnace charge may be relied upon to reduce such compound. In the latter case, the furnace charge will contain sufficient carbon to accomplish both the reduction of the manganese-molybdenum-sulfid compound and to satisfy the usual requirement in the manufacture of the steel. When the molybdenum is recovered in this manner it alloys directly with the steel.

In actual practice of the invention it has been found that molybdenum and ferro-mo-

lybdenum may be readily produced containing less than 0.10% sulfur. The materials utilized in the process are abundant and cheap, and the heat required for carrying out the process is very small due to the exothermic character of the reaction. All of these considerations contribute to the practical and economic character of the process, by which large quantities of molybdenum may be recovered for the rapidly increasing uses to which it is being put.

We claim:

1. A step in the process of recovering molybdenum from molybdenite, which consists in causing an oxid of manganese to react with molybdenite.

2. The process of recovering molybdenum from molybdenite, which consists in causing an oxid of manganese to react with molybdenite in the presence of a reducing agent.

3. The process of recovering molybdenum from molybdenite, which consists in causing manganese dioxide to react with molybdenite in the presence of carbon.

4. The process of producing ferro-molybdenum directly from molybdenite, which consists in causing an oxid of manganese to react with molybdenite in the presence of iron and a reducing agent.

5. The process of recovering metal from a sulfid ore thereof, which consists in causing an oxid of manganese to react with the sulfid ore in the presence of a reducing agent.

In testimony whereof, we have hereunto set our hands.

GEORGE W. SARGENT.  
JOSEPH W. WEITZENKORN.

Witnesses:

MARX HERSCHE,  
WM. H. WEIS.